

# United States Patent Office

2,918,395

Patented Dec. 22, 1959

1

2,918,395

## METHOD OF IMPREGNATING PROTECTIVE CLOTHING

Souren Z. Avedikian, Larchmont, N.Y., assignor to the United States of America as represented by the Secretary of War in trust

No Drawing. Application February 12, 1942  
Serial No. 430,690

16 Claims. (Cl. 117—161)

(Granted under Title 35, U.S. Code (1952), sec. 266)

The invention described herein may be manufactured and used by or for the Government for governmental purposes, without the payment to me of any royalty thereon.

This invention relates generally to certain improvements in protective clothing adapted to give protection against mustard gas and like chemical warfare vesicants, and to certain improvements in methods of making such protective clothing.

More particularly, this invention relates to the type of protective clothing known to those skilled in the art as "permeable protective clothing." This type of protective clothing is permeable to air and moisture and is adapted to have substantially the same wearing characteristics as ordinary clothing. Such permeable protective clothing is distinguished from the other recognized type of protective clothing which is known to those skilled in the art as "impermeable protective clothing." This latter type of protective clothing is impervious to all gases and cannot be worn for long periods of time because it does not permit body perspiration. Impermeable protective clothing is used on a small scale in decontamination work where high vesicant concentrations are encountered.

It has been found that mustard gas and like vesicants can be rendered substantially harmless by halogenation or chlorination so as to convert the vesicant agents into non-irritant products. A number of organic compounds containing available halogen atoms are known which, in various degrees, are capable of chlorinating mustard gas. The chloramines containing available chlorine are, as a class, suitable for this purpose. When these compounds are used as the active agents in protective clothing they are usually referred to as impregnates. The following table is a list of a number of compounds which have been used or suggested as impregnating agents for protective clothing:

2

Of the foregoing compounds, bis 2,4,6-trichlorophenyl chlorurea has been found to be particularly well suited as an impregnating agent.

However, considerable difficulty has been encountered in incorporating the impregnating agents into, or binding them to, fabric or cloth so as to provide satisfactory protective clothing which closely resembles ordinary untreated clothing. Various types of binders for the impregnates have been suggested, none of which has proven entirely satisfactory. The principal objections to protective clothing provided heretofore have been that: (1) it was tacky and sticky so as to be uncomfortable to put on and wear; (2) considerable shrinkage occurred when a garment was treated so as to convert it into protective clothing; and (3) the protective clothing deteriorated appreciably during storage and repeated washing. In addition to the foregoing objectionable properties of protective clothing, heretofore it was necessary to carry out the impregnation treatment at elevated temperatures.

Accordingly, a primary object of this invention, generally stated, is the provision of protective clothing of the type described wherein: (1) tackiness or stickiness is substantially eliminated; (2) which is free from shrinkage; and (3) which retains its initial high protective property in a high degree without deterioration over long periods of time even when subjected to repeated washings. Another important object of this invention is the provision of a method of making protective clothing without shrinkage of the fabric or garment during treatment.

Still another important object of this invention is the provision of a method of impregnating fabric or clothing at ordinary room temperatures so as to render the same impermeable to mustard gas and the like.

Other objects of my invention will, in part, be obvious, and in part appear hereinafter.

In brief, the invention involves the use of a binder comprising a vinyl type polymerization product, or a so-called "Vinylite," and a suitable plasticizer therefor, to bind and incorporate an impregnating agent or anti-vesicant agent into clothing or fabric. Specifically, it has been found that a binder comprising the polyvinyl acetate polymerization product known commercially as "Vinylite A" (Carbide and Carbon Chem. Corp.) and dibutyl phthalate as a plasticizer therefor, is particularly well adapted to bind and incorporate the impregnating agent, bis 2,4,6-trichlorophenyl chlorurea, into fabric or clothing so as to provide superior protective clothing and garments, highly resistant to mustard gas and like vesicants. Protective clothing made with this combination

| Name                                              | Formula                                                                                                      | Percent Active Chlorine |
|---------------------------------------------------|--------------------------------------------------------------------------------------------------------------|-------------------------|
| Aceto 2,4,6-trichlorophenyl chloramide            | $\text{CH}_3\text{CON}(\text{Cl})\text{C}_6\text{H}_3\text{Cl}_3$                                            | 12.99                   |
| Benz 2,4,6-trichlorophenyl chloramide             | $\text{C}_6\text{H}_5\text{CON}(\text{Cl})\text{C}_6\text{H}_3\text{Cl}_3$                                   | 10.59                   |
| p-Brombenzo 2,4,6-trichlorophenyl chloramide      | $\text{BrC}_6\text{H}_4\text{CON}(\text{Cl})\text{C}_6\text{H}_3\text{Cl}_3$                                 | 8.57                    |
| Benz 2,4-dichlorophenyl chloramide                | $\text{C}_6\text{H}_5\text{CON}(\text{Cl})\text{C}_6\text{H}_3\text{Cl}_2$                                   | 11.80                   |
| Aceto 2,4-dichlorophenyl chloramide               | $\text{CH}_3\text{CON}(\text{Cl})\text{C}_6\text{H}_3\text{Cl}_2$                                            | 14.87                   |
| Stear 2,4,6-trichlorophenyl chloramide            | $\text{C}_{17}\text{H}_{35}\text{CON}(\text{Cl})\text{C}_6\text{H}_3\text{Cl}_3$                             | 7.13                    |
| Palmito 2,4,6-trichlorophenyl chloramide          | $\text{C}_{15}\text{H}_{31}\text{CON}(\text{Cl})\text{C}_6\text{H}_3\text{Cl}_3$                             | 7.54                    |
| Benzene sulfone benzyl chloramide                 | $\text{C}_6\text{H}_5\text{SO}_2\text{N}(\text{Cl})\text{CH}_2\text{C}_6\text{H}_5$                          | 12.59                   |
| 2,3,5,6-tetrachlorophenylene bis-aceto chloramide | $\text{C}_6\text{Cl}_4(\text{CH}_3\text{CONCl})_2$                                                           | 17.78                   |
| 2,5-dichlor 4-phenylene bis-aceto chloramide      | $\text{C}_6\text{Cl}_2\text{Cl}_2(\text{CH}_3\text{CONCl})_2$                                                | 21.50                   |
| 4,6-dichlor 3-phenyl bis-aceto chloramide         | $\text{C}_6\text{Cl}_2\text{Cl}_2(\text{CH}_3\text{CONCl})_2$                                                | 21.50                   |
| Terephthal bis-2,4,6-trichlorophenyl chloramide   | $\text{C}_6\text{H}_4(\text{CONCl})_2\text{C}_6\text{H}_3\text{Cl}_3$                                        | 11.98                   |
| Phthal bis-2,4,6-trichlorophenyl chloramide       | $\text{C}_6\text{H}_4(\text{CONCl})_2\text{C}_6\text{H}_3\text{Cl}_3$                                        | 11.98                   |
| Bis-2,4,6-trichlorophenyl chlorurea               | $(\text{C}_6\text{H}_3\text{Cl}_3\text{NCl})_2\text{CO}$                                                     | 14.54                   |
| Dibenzene sulfonyl ethylene dichloradiamide       | $\text{C}_6\text{H}_5\text{SO}_2\text{N}(\text{Cl})\text{CH}_2\text{CH}_2\text{NClSO}_2\text{C}_6\text{H}_5$ | 17.33                   |
| Phthal-chloramide                                 | $\text{C}_6\text{H}_4(\text{CO})_2\text{NCl}$                                                                | 19.54                   |
| Chlorortho benzoic sulfonide                      | $\text{C}_6\text{H}_3\text{CO}(\text{SO}_2)\text{NCl}$                                                       | 16.30                   |
| Quinone dichlorimid                               | $\text{C}_6\text{H}_4(\text{NCl})_2$                                                                         | 40.05                   |
| Chlorsuccinimid                                   | $(\text{CH}_2\text{CO})_2\text{NCl}$                                                                         | 26.50                   |
| Dibenzoyl ethylene dichloradiamine                | $\text{C}_6\text{H}_5\text{CON}(\text{Cl})\text{CH}_2\text{CH}_2\text{NClCOOC}_6\text{H}_5$                  | 21.04                   |
| Benzoyl chlorcarbamide                            | $\text{C}_6\text{H}_5\text{CONHCONHCl}$                                                                      | 17.86                   |
| Dibenzoyl dichlorcarbamide                        | $(\text{C}_6\text{H}_5\text{CONCl})_2\text{CO}$                                                              | 20.75                   |
| Iodobenzene dichloride                            | $\text{C}_6\text{H}_5\text{Cl}_2$                                                                            | 25.83                   |
| "Halazone"                                        | $\text{COOHCH}_2\text{C}_6\text{H}_4\text{SO}_2\text{NCl}_2$                                                 | 26.26                   |
| Bis(dichlorophenylchlor)urea                      | $(\text{C}_6\text{H}_3\text{Cl}_3\text{NCl})_2\text{CO}$                                                     | 16.98                   |

of binder and impregnating agent is particularly distinguished by the absence of shrinkage on impregnation, its freedom from stickiness and tackiness, and its high resistance to deterioration.

For a more complete understanding of the nature and scope of this invention reference may be had to the following detailed illustrative description thereof.

Any ordinary type of fabric, such as cotton, wool, or mixtures thereof, may be treated according to this invention either before or after it has been made into garments. The impregnating agent and binder may be applied to the fabric or clothing in the form of a solution thereof in a volatile solvent. A solution of the following composition has given good results in practice:

"Vinylite A" (Carbide and Carbon Chem. Corp.) -- 1% by weight.  
 Plasticizer ----- 1% by weight (dibutyl phthalate).  
 Volatile solvent ----- 91% by weight (acetylene tetrachloride).  
 Protective agent ----- 7% by weight (bis 2-4-6 trichlorphenyl chlorurea).

It will be understood that the foregoing composition may be varied within limits and that the constituents may be replaced by various equivalent materials. For example, the acetylene tetrachloride may be replaced by chlorobenzene or any other suitable volatile solvent in which the ingredients are sufficiently soluble and which is inert thereto. Likewise the bis 2-4-6 trichlorphenyl chlorurea may be entirely or partially replaced by bis dichlorphenyl chlorurea. The Vinylite may be used in amounts up to 5% by weight, or even greater, and the protective agent may be used in amounts up to the limit of its solubility in the solvent, and even in amounts exceeding its solubility if measures are taken to thoroughly agitate the mixture so as to maintain an intimate mixture and dispersion of the solid phase throughout the solution during impregnation.

One satisfactory method of treating fabric or garments with the above or equivalent solutions is to immerse the fabric or garments in a bath of the solution at room temperature so as to thoroughly wet the same. Then the fabric or garments may be removed from the bath and excess liquid removed therefrom either by wringing or centrifuging the same. Thereafter, the fabric or garments may be allowed to dry so as to complete the removal of the volatile solvent and leave the impregnating agent and binder firmly incorporated in the fibers.

Care should be taken to remove as much of the excess liquid as can be conveniently done by wringing or centrifuging so as to keep the increase in weight of the fabric or garment due to impregnation to a minimum and at the same time prevent the unnecessary closing off of the interstices and openings between the fibers.

It will be understood that certain other methods and techniques may be employed to treat fabric and clothing with the impregnating solutions.

Cloth impregnated with a solution having the composition outlined above and according to the foregoing method will have the following approximate composition with regard to the materials added:

Total materials added, (i.e., increase in 25 to 28% of the weight of untreated cloth) ----- original weight.

Percentage of binder and protective agent in treated cloth ----- 20-22%.  
 Percentage of binder ----- 3-5%.  
 Percentage of protective agent ----- 17+%.

The unexpected resistance to deterioration of protective clothing made according to this invention is thought to be due in large measure to the fact that the Vinylite type of binder not only serves to bind the protective

agent into the fabric, but that it also serves as a protective agent for the fibers of the clothing or fabric.

Since certain changes may be made in the foregoing compositions, percentages, and techniques of application 5 without departing from the scope of the invention, it is intended that all matter described above be interpreted as illustrative and not in a limiting sense.

I claim:

- 10 1. The method of providing, without substantial shrinkage, non-tacky, air-permeable protective fabric and clothing resistant to mustard gas and like vesicants susceptible of being rendered non-vesicant by chlorination, which comprises, impregnating the fabric or clothing with bis 2,4,6-trichlorphenyl chlorurea incorporated in a binder comprising a vinyl ester polymerization product.
- 15 2. The method of providing, without substantial shrinkage, non-tacky, air-permeable protective fabric and clothing resistant to mustard gas and like vesicants susceptible of being rendered non-vesicant by chlorination, 20 which comprises, impregnating the fabric or clothing with bis 2,4,6-trichlorphenyl chlorurea incorporated in a binder comprising a vinyl ester polymerization product and a plasticizer therefor.
- 25 3. The method of providing, without substantial shrinkage, non-tacky, air-permeable protective fabric and clothing resistant to mustard gas and like vesicants, susceptible of being rendered non-vesicant by chlorination, 30 which comprises, impregnating the fabric or clothing with bis 2,4,6-trichlorphenyl chlorurea incorporated in a binder comprising a vinyl ester polymerization product and di-butyl phthalate.
- 35 4. The method providing, without substantial shrinkage, non-tacky, air-permeable protective fabric and clothing resistant to mustard gas and like vesicants susceptible of being rendered non-vesicant by chlorination, 30 which comprises, impregnating the fabric or clothing at room temperature with bis 2,4,6-trichlorphenyl chlorurea incorporated in a binder comprising a vinyl ester polymerization product and a plasticizer therefor.
- 40 5. The method of providing, without substantial shrinkage, non-tacky, air-permeable protective fabric and clothing resistant to mustard gas and like vesicants, which comprises, wetting fabric or clothing with a solution of bis 2,4,6-trichlorphenyl chlorurea and a binder comprising a vinyl ester polymerization product and di-butyl phthalate, removing excess of said solution from the wetted fabric or clothing, and drying the treated fabric or clothing.
- 45 6. The method of providing, without substantial shrinkage, non-tacky, air-permeable protective fabric and clothing resistant to mustard gas and like vesicants, which comprises, wetting fabric or clothing at room temperature with an intimate mixture of bis 2,4,6-trichlorphenyl chlorurea and a binder comprising polyvinyl acetate and a plasticizer therefor, in acetylene tetrachloride, removing excess of said intimate mixture from the wetted fabric or clothing, and drying the treated fabric or clothing so as to remove acetylene tetrachloride solvent therefrom.
- 50 60 7. The method of providing, without substantial shrinkage, non-tacky, air-permeable protective fabric and clothing resistant to mustard gas and like vesicants, which comprises, wetting fabric or clothing at room temperature with a solution comprising by weight about 7% of bis 2,4,6-trichlorphenyl chlorurea, about 2% by weight of a binder comprising approximately equal parts of a vinyl ester polymerization product and dibutyl phthalate plasticizer therefor in about 91% by weight of acetylene tetrachloride, removing excess of said solution 65 from the wetted fabric or clothing, and drying the treated fabric or clothing so as to remove acetylene tetrachloride solvent therefrom.
- 70 8. The method of providing, without substantial shrinkage, non-tacky, air-permeable protective fabric and clothing resistant to mustard gas and like vesicants, 75

which comprises, wetting fabric or clothing at room temperature with a solution comprising by weight about 7% of bis 2,4,6-trichlorphenyl chlorurea, about 2% by weight of a binder comprising approximately equal parts of polyvinyl acetate and dibutyl phthalate plasticizer therefor, in about 91% by weight of acetylene tetrachloride, removing excess of said solution from the wetted fabric or clothing, and drying the treated fabric or clothing so as to remove acetylene tetrachloride solvent therefrom.

9. Protective clothing impermeable to mustard gas and like vesicants susceptible of being rendered non-vesicant by chlorination, and characterized by being non-tacky, air-permeable, and relatively comfortable to wear, and made from fabric impregnated with bis 2,4,6-trichlorphenyl chlorurea incorporated in a binder comprising a vinyl ester polymerization product.

10. Protective clothing impermeable to mustard gas and like vesicants susceptible of being rendered non-vesicant by chlorination, and characterized by being non-tacky, air-permeable, and relatively comfortable to wear, and made from fabric impregnated with bis 2,4,6-trichlorphenyl chlorurea incorporated in a binder comprising a vinyl ester polymerization product and plasticizer therefor.

11. Protective clothing impermeable to mustard gas and like vesicants susceptible of being rendered non-vesicant by chlorination, and characterized by being non-tacky, air-permeable, and relatively comfortable to wear, and made from fabric impregnated with bis 2,4,6-trichlorphenyl chlorurea incorporated in a binder comprising a vinyl ester polymerization product and dibutyl phthalate.

12. Protective clothing impermeable to mustard gas and like vesicants susceptible of being rendered non-vesicant by chlorination, and characterized by being non-tacky, air-permeable, and relatively comfortable to wear, and made from fabric impregnated with bis 2,4,6-trichlorphenyl chlorurea incorporated in a binder comprising a vinyl ester polymerization product and dibutyl phthalate, said bis 2,4,6-trichlorphenyl chlorurea being present in an amount equal to about 15% to 17% of the weight of the fabric, and said binder being present in an

amount equal to about 3% to 5% of the weight of the fabric.

13. A fabric impregnating composition for rendering fabric and clothing impermeable to mustard gas and like vesicants susceptible of being rendered non-vesicant by chlorination but permeable to air, which comprises, an intimate mixture of bis 2,4,6-trichlorphenyl chlorurea and a binder comprising a vinyl ester polymerization product and plasticizer therefor, in a volatile solvent.

14. A fabric impregnating composition for rendering fabric and clothing impermeable to mustard gas and like vesicants susceptible of being rendered non-vesicant by chlorination but permeable to air, which comprises an intimate mixture of bis 2,4,6-trichlorphenyl chlorurea and a binder comprising polyvinyl acetate and a plasticizer therefor, in a volatile solvent.

15. A fabric impregnating composition for rendering fabric and clothing impermeable to mustard gas and like vesicants susceptible of being rendered non-vesicant by chlorination but permeable to air, which comprises an intimate mixture of bis 2,4,6-trichlorphenyl chlorurea and a binder comprising polyvinyl acetate and dibutyl phthalate, in acetylene tetrachloride.

16. A fabric impregnating composition for rendering fabric and clothing impermeable to mustard gas and like vesicants susceptible of being rendered non-vesicant by chlorination but permeable to air, which comprises a solution of about 7% by weight of bis 2,4,6-trichlorphenyl chlorurea and about 2% by weight of a binder comprising approximately equal parts of polyvinyl acetate and dibutyl phthalate, in about 91% by weight of acetylene tetrachloride.

35 References Cited in the file of this patent

UNITED STATES PATENTS

2,173,781 Gibells \_\_\_\_\_ Sept. 19, 1939

FOREIGN PATENTS

40 373,947 Great Britain \_\_\_\_\_ June 2, 1932  
448,164 Great Britain \_\_\_\_\_ June 3, 1936  
486,162 Great Britain \_\_\_\_\_ May 31, 1938